

# UNITED STATES PATENT OFFICE.

ARTHUR J. WEED, OF NEW YORK, N. Y., ASSIGNOR OF ONE-HALF TO EUGENE W. CALDWELL, OF NEW YORK, N. Y.

## PERMANENT MAGNET AND PROCESS OF MAKING THE SAME.

1,183,258.

Specification of Letters Patent.

Patented May 16, 1916.

No Drawing.

Application filed June 21, 1909. Serial No. 503,330.

*To all whom it may concern:*

Be it known that I, ARTHUR J. WEED, a citizen of the United States, and resident of the city, county, and State of New York, have made certain new and useful Inventions Relating to Permanent Magnets and Processes of Making the Same, of which the following is a specification.

This invention relates to permanent magnets and processes of making the same, especially by the treatment of iron castings at a low heat in the presence of cobalt salts or compounds, preferably in a closed chamber.

15 Iron and other magnetic materials, such as iron castings of various grades especially hard low grade cast iron, may be given a high degree of permanent magnetism after first treating them in the proper way with 20 suitable cobaltous or other similarly acting sensitizing material. For this purpose the iron castings may be heated for a sufficient time to a suitable temperature capable of effecting the desired sensitizing action preferably for several hours or so to a temperature somewhat below that of a visible red 25 heat in the presence of suitable cobaltous sensitizing material which may be conveniently effected while the iron, for instance, 30 is surrounded by sand or the like in a closed chamber. The sensitizing material which may with good effect be in the form of a mixture of about equal parts of black oxid of cobalt and red cobaltous sulfate may be 35 applied to the iron castings by any suitable varnish or other medium in which the finely powdered cobaltous material is incorporated. With small castings of a few pounds, such as are suitable for use in magneto machines 40 the cobaltous material may be applied to about the thickness of an ordinary coat of paint or the magnet after having been varnished with shellac or the like may be dipped into a finely pulverized mixture of 45 the cobalt sensitizing salts or the like, or they may be brought into sufficiently close contact with the iron during the treating process. Thereafter the magnet may be covered with sand in a cast iron or other 50 suitable treating chamber and kept at a dull heat just below a visible red and then allowed to slowly cool which has a desirable annealing and softening action with many grades of hard cast iron so that they may

be more easily machined and finished. The sensitized iron castings may be cleaned and magnetized in any desired manner. This sensitizing treatment seems to effect some combination or union of the cobaltous sensitizing material with the iron or to effect some molecular rearrangement of its constituents so as to render it much more susceptible to and capable of permanently retaining considerable magnetic properties. Many other forms of cobalt material, such as metallic cobalt or the chlorids, for instance, seem to have a similar sensitizing action on ferreous magnetic material and may be used either alone or in combination with the sensitizing materials indicated.

Having described this invention in connection with a number of illustrative ingredients, proportions, steps and methods of treatment, to the details of which disclosure the invention is not of course to be limited, what is claimed as new and what is desired to be secured by Letters Patent is set forth in the appended claims.

1. A permanent magnet composed of annealed cast iron which contains, in its superficial portions, a trace of cobaltous material, whereby it is capable of retaining magnetism to a considerably higher degree than similar cast iron which contains no such cobaltous material.

2. A permanent magnet composed of annealed cast iron capable of being easily machined and finished and which contains, in its superficial portions, at least a trace of cobaltous sensitizing material, whereby it is capable of retaining magnetism to a considerably higher degree than similar cast iron which contains no such cobaltous material.

3. The process of forming a permanent magnet capable of retaining a high degree of magnetization which consists in bringing sensitizing material into intimate contact with a hard iron casting and in heating the same at a temperature approximately that of a visible red heat in a substantially closed treating chamber and in slowly cooling and annealing said casting to facilitate its machining and finishing and in magnetizing said casting, substantially as described.

4. The process of forming a permanent magnet capable of retaining a high degree of magnetization which consists in bringing co-

balt sensitizing material comprising substantially equal parts of cobalt oxid and cobaltous sulfate into intimate contact with a hard iron casting and in heating the same for several hours at a temperature slightly below a visible red heat in a substantially closed treating chamber and in slowly cooling and magnetizing said casting.

5. The process of forming a permanent magnet capable of retaining a high degree of magnetization which consists in applying cobalt sensitizing material to an iron casting and in heating said casting for a considerable time in a substantially closed chamber at a 10 temperature somewhat below a visible red heat and in cooling and magnetizing said casting.

6. The process of forming a permanent magnet capable of retaining a considerable 20 degree of magnetization which consists in heating an iron casting for a considerable time in intimate contact with cobalt sensitizing material and in cooling and magnetizing said casting.

25 7. The process of forming a permanent magnet capable of retaining a high degree of magnetization which consists in heating a ferreous casting for a considerable time at a sensitizing temperature somewhat below a 30 visible red heat in the presence of cobalt

sensitizing material and in magnetizing said casting.

8. The process of treating ferreous magnetic material so as to be capable of retaining a high degree of magnetization which consists in heating said material for a considerable time at a sensitizing temperature somewhat below a visible red heat in the presence of cobalt sensitizing material.

9. The process of softening an iron casting and rendering the same capable of retaining a high degree of magnetization which consists in heating said casting for a considerable time at a sensitizing temperature somewhat below a visible red heat in 45 the presence of cobalt sensitizing material and in gradually cooling said casting.

10. The process of rendering ferreous magnetic material capable of retaining a high degree of magnetization which consists in heating said material for a considerable time at a sensitizing temperature capable of rendering active cobalt sensitizing substance while said material is in the presence of said sensitizing substance and in cooling said 55 material.

ARTHUR J. WEED.

Witnesses:

HARRY L. DUNCAN,  
JESSIE B. KAY.